

## UNITED STATES PATENT OFFICE

2,105,310

## AGGLUTINANT

Isidor Chesler, New York, N. Y., assignor to Eagle  
Pencil Company, a corporation of DelawareNo Drawing. Application April 14, 1934,  
Serial No. 720,573

22 Claims. (Cl. 106—40)

While my present invention is more particularly concerned with agglutinating materials useful in various arts and of particular utility as the binder in the art of colored pencil or crayon leads or rods.

Among the objects of the invention are to provide an agglutinant useful for a lead or rod of the non-calcined type, which admits of making the same in any desired length, shape or color, including also black and white, of any desired hardness or softness, which imparts to the lead properties such that, even in small diameters it has tensile and shearing strength, as well as elasticity of high order, and admits of being sharpened to a point like ordinary graphite pencil leads and the strength and writing qualities of which are not adversely affected by the glue used for bonding the writing rod into a conventional wooden case.

Another object is to provide a binder for a pencil or crayon lead or rod of the above type, the use of which affords sufficient penetrability to the lead to permit incorporation therein of waxy or fatty material or both, which determines certain of the writing qualities of the rod.

Another object is to provide an agglutinant more especially suitable as the binder of the lead or crayon-rod composition, which while contributing largely to the foregoing desired properties, is itself neither too horny nor tough, but wears readily and uniformly with the writing end of the pencil rod as the latter is consumed in use.

Another object is to provide an agglutinant or binder of composite character including both a gummy mass acting as an adhesive binder, and stringy particles acting mechanically primarily to reinforce the rod.

Another object is to provide an agglutinant or binder of the above character which will not powder or harden or otherwise deteriorate with age to such extent as to impair its usefulness, and which requires no highly volatile nor inflammable solvents and thus obviates the expense and the danger due to the use of such solvents.

Other objects will be in part obvious and in part pointed out hereinafter.

According to the invention, the agglutinating material is largely or wholly composed of etherized cellulose of solubility in water for example, to a degree less than that of completely methylated cellulose and to a degree greater than completely ethylated cellulose.

The preferred agglutinant or binder has a relatively high viscosity, suggesting in part at least a colloidal suspension rather than a true solution, the agglutinant or binder being preferably not too

readily water soluble, and not entirely dissolved in cold water.

Alkyl-ethers of cellulose wholly devoid of methyl radicals, as for instance, completely ethylated cellulose are, in general, substantially insoluble in water and the use of non-aqueous solvents, such as alcohol, glycerin, acetone or the like for preparing the paste for lead or crayon manufacture, in general, yields a product lumpy, brittle, hygroscopic or otherwise objectionable for practical purposes. Solubility in water generally increases with an increase of methyl radicals in the etherized cellulose, completely methylated or tri-methyl cellulose having maximum water solubility, and in solution presenting a substantially homogeneous gummy substance from which a film having limited elasticity, resiliency and tensile strength may be formed, which while superior to gum tragacanth as a binder for lead and crayon rod compositions is inferior to the preferred mixed ether of cellulose to be described hereinafter.

The preferred agglutinating material used for the purpose of this invention is not entirely homogeneous, for when thoroughly soaked in water, there is present as insoluble or colloidal or colloidized material, small portions of relatively insoluble or but partially soluble particles of a stringy character, disseminated throughout the mass.

The desired substance or binder of non-homogeneous or heterogeneous character, in part gummy and in the dissolved state, and in part stringy and but partially or imperfectly dissolved, is composed preferably of mixed etherized cellulose, which may, on the one hand be prepared as a physical admixture of diverse ethers of cellulose having the required diverse properties, or, on the other hand, may result from controlled etherification with diverse radicals, of one and the same mass of cellulose, which previously has been subjected to a mercerizing treatment.

A specific agglutinant or binder, according to the invention, consists largely of di-methyl ethyl ether of cellulose, (that is, cellulose in which two of the replaceable hydroxyls have been substituted by methyl group, and the other hydroxyl by ethyl group), substantially soluble in water, to yield the gummy medium, and this may or may not be admixed, depending upon the particular results to be obtained in the finished products, with other ethers of cellulose, poorer or lacking in the methyl radical and substantially insoluble in water, which constitutes the stringy ingredient of the binder.

Where as ordinarily preferred, it is desired to

- produce the mixed cellulose ether by one operation, in a single series of etherizing steps as in the formation, for instance, of an etherized cellulose containing both methyl and ethyl there-  
5 in, as substituent groups, that is, a methyl-ethyl cellulose, purified cellulose, is treated with caustic soda, which operation mercerizes or renders the cellulose more susceptible to etherization, it being well known to those skilled in the art, that  
10 mercerized cellulose or alkaline cellulose is more susceptible to etherification than is normal, original or unmodified cellulose. Thereupon the mercerized cellulose is etherized by treating with esters such as the chlorides or sulphates having  
15 the desired alkyl radicals. Preferably a mixture is used of like esters of methyl and of ethyl to produce the mixed methyl ethyl cellulose, as a mixture of dimethyl sulphate with diethyl sulphate.  
20 While the above description may be sufficient to enable those skilled in the art to prepare the agglutinant or binder of the present invention, a detailed illustrative specification will now be given, to assure compliance with the statutory  
25 requirements.

An alkali-cellulose (soda cellulose) is first prepared from the purified cellulose obtained, either purified wood pulp or purified cotton pulp and preferably of as high alphacellulose content as  
30 possible, (such as the cellulose found most suitable for xanthating in the formation of viscose rayon) by treatment with sodium hydroxide solution of 18-20 per cent absolute NaOH or higher, for about 2 hours at 17-22 degrees C. The alkali-cellulose is then shredded or otherwise subdivided into small particles, and then intimately admixed for several hours with finely powdered solid sodium hydroxide, 20 to 50 per cent of the weight of the original cellulose taken being employed, and as free from sodium carbonate and other impurities as possible. The length of time required, temperatures and concentrations for mixing are primarily dependent upon the solubility, viscosity and other physical characteristics  
40 desired in the final product. This finely divided mass is then placed in a pressure container, if to be alkylated with a haloid ester as methyl chloride or ethyl chloride, or in an open container, if to be alkylated with a mixture of di-  
45 methyl sulphate and diethyl sulphate, either container being preferably provided with efficient stirring apparatus, and heated at from 100-140 degrees C. from one to four hours. The temperature of the reacting mass, after the addition of  
50 a proportion of methyl ester and ethyl ester, depends upon the degree of etherification, and the proportion of methyl to ethyl desired in the finished etherized cellulose. A desirable result is obtained by taking two parts by weight of  
55 the methyl ester to one part of the ethyl.

At the completion of the etherification step, the mass is then precipitated, as by the addition of water or of brine, depending upon the degree of solubility in water of the etherized cellulose, or  
60 if methyl and ethyl chlorides are used as etherifying agents, the excess of alkyl chloride may be removed by distillation. The crude mass is washed with brine or cold water to remove further amounts of reactants, if desired, and then  
65 dried at a comparatively low temperature.

The product after washing and drying is, in general, a flocculent substance, which when treated with water assumes a fluid, gummy consistency, but is not entirely homogeneous, since  
75 it has distributed therein, the desired small

stringy particles that are relatively unaffected or little affected by water. The gummy mass of the water-treated flocculent ether cellulose is probably largely di-methyl ethyl cellulose, which may have admixed therewith small proportions 5 of trimethyl cellulose, and other bodies of a cellulose etherized character. The stringy water-insoluble particles are probably ethers of cellulose having not less than two ethyl radicals and probably having to some extent ethyl radicals 10 substituted for all replaceable hydroxyls. The precise chemical composition of the agglutinant product is not known, but it seems probable that it consists of or contains various ethers of cellulose obtainable from the ingredients used, and 15 that while most of the cellulose is completely etherized, a portion thereof is incompletely etherized. The stringy particles may in whole or in part be unetherized cellulose or other fiber. Preferably, the agglutinant after treatment with 20 water has 15 to 25 per cent by weight of the insoluble, incompletely soluble or difficultly soluble stringy ingredient therein.

The mixed ether cellulose of which the foregoing is a specific example may for present purposes consist of any of a relatively wide variety of ingredients, preferably, however, including some alkyl radical of lower order. Among the various ethers which serve for the purpose are mixed alkyl-cellulose, mixed alkyl-aryl cellulose, 30 and mixed alkyl-aralkyl cellulose.

While unlike the other ethers of cellulose the aryl cellulose is not to applicant's knowledge in commercial use at the present time, it is applicable for present purposes as herein set forth and 35 as a chemical individual is known in the literature as appears from the following reference,— A. Nastukoff, Journal of Russian Physical and Chemical Society, 1902, volume 39, pages 1109-35; Biochemisches Handlexikon, 1911, volume 2, page 40 232.

A preferred mixed alkyl-cellulose is the di-methyl-ethyl cellulose above described; an example of a mixed alkyl-aryl cellulose is di-methyl-phenyl cellulose; and of a mixed alkyl-aralkyl 45 compound is di-methyl-benzyl cellulose. In each case, the bulk of the mixed cellulose ether is preferably to contain at least one and preferably two methyl radicals, in association with a member or members of one or more of other groups 50 of radicals, including those enumerated above.

For a more complete understanding of a preferred application of the agglutinant, the structure and method of preparation of my new pencil and crayon rods therewith, will now be set forth. 55

According to the invention, the etherized cellulose to be used as agglutinant is soaked in water one or two days before use, preferably in a tinned copper vessel inert to the agglutinant.

The base mixture used for the lead or crayon composition comprises a filler such as ground china clay and a pigment such as miliot blue ground wet, comminuted, filter pressed and air dried, and after admixture with stearic acid and further crushing, admixed with calcium stearate 65 and still further mixed. Thereupon the desired proportion of water soaked agglutinant is added, together with enough water to bring the mass to the desired consistency or plasticity. Experience has shown that a preferred moisture 70 content, determinable by analysis of a specimen will range around 20 to 25 per cent.

The mixture of the batch is now ground, compressed and kneaded by use of a series of appropriate mills for securing a homogeneous in- 75

timately mixed and tough dough, which is thereupon hammered into cylinders and forced through perforated plates and re-compressed. Finally the dough is forced through dies of the proper calibre 5 to produce the rod-like lead product. In this operation, the stringy particles in the binder appear to become oriented substantially longitudinally of the rod and thus intermingled and intermeshed, thereby materially augmenting the 10 mechanical strength of the product.

The lead rods are dried in racks according to familiar practice, including covering the leads with boards to prevent warping thereof, first at room temperature, then maintaining the leads 15 for a week or more in a drying chamber at a temperature of 120 degrees F. or thereabouts, with the application of air in motion, until the moisture content of leads on test is found to be very low, whereupon the leads are cut to size.

20 The rod tightly compacted by the process above set forth develops or has therein minute pores, probably due to the escape therefrom of water evaporated in the drying operation. For all purposes except where the rods are made with water soluble dyes, such as are used for copying pencils or the like, the rods are subjected to a waxing operation now to be set forth. For such purposes, the dried rods after reheating to approximately the temperature of the molten wax to be used 25 30 in the next step are then immersed for a period of some hours in a mixture of waxes, or material of a waxy nature, ordinarily equal parts of stearic acid and carnauba wax, preferably at a temperature of 180 to 190 degrees F. The dried rod has sufficient porosity to permit such melted waxy substances thoroughly to permeate the same, under the conditions of treatment, that is, to substantially fill all voids left in the rods by the evaporation of the water, and to fill the interstices in the stringy ingredient of the binder, a penetration attainable with much difficulty, if at all, where the lead has a case-hardened imperforate surface. The thorough wax impregnation results in a lead or crayon rod of excellent 40 45 and uniform writing properties. After cooling, the leads are tested for strength, grade and quality and then preferably glued into the usual wooden sheaths.

The lead has tensile and shearing strength considerably greater than that of the best grades of leads of corresponding size at present on the market, and can be bent through a visible arc before breaking.

The agglutinant when used as the binder for 55 the leads of writing implements, is by no means limited in its application to colored crayons or pencils, but may be used for black leads or for white leads as well.

It will thus be seen that there is herein described an article and composition in which the several features of this invention are embodied, and which article and composition in their action attain the various objects of the invention and are well suited to meet the requirements of practical use.

As many changes and variations may be made in the above article and composition, and many apparently widely different embodiments of this invention may be made without departing from 70 the scope thereof, it is intended that all matter contained in the above description, shall be interpreted as illustrative and not in a limiting sense.

What I claim as new and desire to secure by 75 Letters Patent is:—

1. A physically and chemically heterogeneous agglutinating material substantially composed of diversely and partially etherized cellulose of the character, presenting in aqueous admixture, small stringy structures of less soluble character 5 distributed in a more soluble homogeneous carrier.

2. A physically and chemically heterogeneous agglutinating material comprising compound incompletely etherized cellulose, including a portion 10 soluble in water and a portion incompletely soluble therein and in the form of small stringy particles, distributed in said first portion.

3. A physically and chemically heterogeneous agglutinating material comprising mixed partially 15 etherized cellulose presenting in aqueous admixture, a carrier of water-soluble etherized cellulose, and small stringy particles therein of etherized cellulose, not entirely soluble in water, said stringy ingredient being by weight substantially fifteen to twenty-five per cent of the mass. 20

4. A physically and chemically heterogeneous agglutinating material comprising a portion soluble in water and a portion incompletely soluble therein and in the form of small stringy particles distributed in said first portion and consisting largely of mixed etherized cellulose in which replaceable hydroxyls in cellulose have substituted therefor to different extents and distribution throughout the mass dissimilar radicals 30 of the classes designated as alkyl, aryl and aralkyl. 25

5. A physically and chemically heterogeneous agglutinating material composed largely of mixed etherized cellulose in which to different extents 35 and distribution throughout the mass methyl is partially substituted for replaceable hydroxyls in cellulose and in which a radical other than methyl is substituted for other replaceable hydroxyls, the whole forming an etherized cellulose 40 partially soluble in water, and containing a portion stringy in character and not dissolving in water.

6. A physically and chemically heterogeneous agglutinating material comprising a portion soluble in water and a portion incompletely soluble therein and in the form of small stringy particles distributed in said first portion consisting of etherized cellulose in which all the replaceable hydroxyls have substituted therefor radicals to 50 different extents and distribution throughout the mass at least two of which are dissimilar and of the classes designated as alkyl, aryl and aralkyl. 45

7. A physically and chemically heterogeneous agglutinating material comprising a portion soluble in water and a portion incompletely soluble therein and in the form of small stringy particles distributed in said first portion and consisting of a cellulose product in which at least one of the hydroxyls is replaced by the methyl radical, and other hydroxyls have substituted therefor to different extents and distribution throughout the mass non-methyl radicals of the classes designated as alkyl, aryl and aralkyl. 55 60

8. A physically and chemically heterogeneous agglutinating material comprising alkylcellulose, having both methyl and ethyl radicals substituted for the replaceable hydroxyls of the original cellulose the resultant product comprising a mixture of various ethyl and methyl compounds 70 of cellulose presenting portions of greater and other portions of lesser solubility.

9. A physically and chemically heterogeneous agglutinating material of etherized cellulose including largely a gummy aqueous solution of sus- 75

- 5 pension richer in methyl radicals and, having interspersed therein stringy, porous non-water soluble particles lower in methyl radicals.
10. A physically and chemically heterogeneous 5 agglutinating material of etherized cellulose including largely a gummy aqueous solution or suspension in which methyl radicals are substituted for most of the replaceable hydroxyls, said solution or suspension having interspersed therein 10 stringy capillary non-water soluble particles of ether cellulose low in methyl radicals.
11. A physically and chemically heterogeneous 15 agglutinating material comprising mixed etherized cellulose presenting a water-soluble, gummy mass the major portion of methylated cellulose having distributed therein small stringy structures of etherized cellulose low in methyl radicals and relatively insoluble in water.
12. A physically and chemically heterogeneous 20 agglutinating material comprising mixed etherized cellulose presenting a water-soluble, gummy mass essentially of methylated cellulose having distributed therein small stringy structures of etherized cellulose relatively insoluble in water, 25 said insoluble particles having two or more radicals selected from the alkyl group, (other than methyl), the aryl and the aralkyl groups.
13. A physically and chemically heterogeneous 30 agglutinating material of mixed alkyl aryl cellulose of a degree of etherification such that a major portion is soluble in water and has interspersed therein stringy particles of ether incompletely soluble in water.
14. A physically and chemically heterogeneous 35 agglutinating material of mixed alkyl aryl cellulose, including at least one methyl radical said material comprising stringy particles of ether incompletely soluble in water interspersed in ether completely soluble in water.
- 40 15. A physically and chemically heterogeneous 40 agglutinating material of mixed alkyl-aryl cellulose containing dimethylphenyl cellulose said material comprising stringy particles of ether incompletely soluble in water interspersed in ether completely soluble in water.
- 45 16. A physically and chemically heterogeneous 45 agglutinating material of mixed alkyl-aryl cellulose essentially of dimethylphenyl cellulose said material comprising stringy particles of ether incompletely soluble in water interspersed in 5 ether completely soluble in water.
17. A physically and chemically heterogeneous 10 agglutinating material comprising a mixed cellulose ether containing an aryl group and alkyl groups, including at least one methyl group said 10 material comprising stringy particles of ether incompletely soluble in water interspersed in ether completely soluble in water.
18. A physically and chemically heterogeneous 15 agglutinating material of mixed alkyl-aralkyl 15 cellulose said material comprising stringy particles of ether incompletely soluble in water interspersed in ether completely soluble in water.
19. A physically and chemically heterogeneous 20 agglutinating material of mixed alkyl-aralkyl 20 cellulose, including at least one methyl radical said material comprising stringy particles of ether incompletely soluble in water interspersed in ether completely soluble in water.
20. A physically and chemically heterogeneous 25 agglutinating material of mixed alkyl-aralkyl 25 cellulose containing dimethylbenzyl cellulose said material comprising stringy particles of ether incompletely soluble in water interspersed in ether completely soluble in water. 30
21. A physically and chemically heterogeneous 35 agglutinating material of mixed alkyl-aralkyl cellulose essentially of dimethylbenzyl cellulose said material comprising stringy particles of ether incompletely soluble in water interspersed in 35 ether completely soluble in water.
22. A physically and chemically heterogeneous 40 agglutinating substance comprising a mixed cellulose ether containing an aralkyl group and dissimilar alkyl groups including at least one methyl group said material comprising stringy particles of ether incompletely soluble in water interspersed in ether completely soluble in water. 45